

# United States Patent

[11] 3,619,238

[72] Inventors **Shiro Kimura;**  
**Teruo Kobayashi; Sadao Ishige, all of**  
**Kanagawa, Japan**

[21] Appl. No. **841,991**

[22] Filed **July 15, 1969**

[45] Patented **Nov. 9, 1971**

[73] Assignee **Fuji Photo Film Co., Ltd.**  
**Kanagawa, Japan**

[32] Priority **July 15, 1968**

[33] **Japan**

[31] **43/49816**

[54] **PRESSURE SENSITIVE COPYING PAPER**  
2 Claims, No Drawings

[52] U.S. Cl. .... **117/36.2,**  
117/36.9, 260/330.5

[51] Int. Cl. .... **B41m 5/22**

[50] Field of Search .... **117/36.2,**  
**36.8, 36.9; 260/330.5**

[56] **References Cited**

UNITED STATES PATENTS

|           |        |              |       |          |
|-----------|--------|--------------|-------|----------|
| 3,491,116 | 1/1970 | Lin          | ..... | 117/36.2 |
| 3,499,902 | 3/1970 | Coles et al. | ..... | 117/36.2 |
| 3,509,174 | 4/1970 | Lin          | ..... | 117/36.8 |

Primary Examiner—Murray Katz  
Attorney—Sughrue, Rothwell, Mion, Zinn & Macpeak

**ABSTRACT:** A pressure sensitive copying paper is prepared using a color former of the general formula



wherein R<sub>1</sub> and R<sub>2</sub> each represents an alkyl group having 1 to 5 carbon atoms or a benzyl group, and X<sub>1</sub>, X<sub>2</sub>, X<sub>3</sub> and X<sub>4</sub> each represents a hydrogen atom, a halogen atom, an alkoxy group or a methyl group. The compound of the above general formula is encapsulated in solution and the thus formed microcapsules are applied to an upper paper. When this upper paper is superimposed over a lower paper coated with an electron acceptable solid acid such as an acid clay, in such a manner that the microcapsule coated surface is in direct contact with the acid coated surface, and pressure applied thereto, a deep reddish purple color is formed in those areas to which pressure has been applied. The color former of the above general formula may also be admixed with yellow orange, or blue color formers to produce black images.

## PRESSURE SENSITIVE COPYING PAPER

The present invention relates to a pressure sensitive copying paper and more particularly to a pressure sensitive copying paper in which color formers are used.

Ordinary pressure sensitive papers are classified into two types, the first of which comprises a combination of a so-called upper paper and a lower paper. The upper paper is prepared by applying to a surface of a support microcapsules containing an organic solvent solution of a substantially colorless organic compound having electron donating and color forming properties (hereinafter referred to as "color former"). The lower paper is prepared by applying an electron acceptable solid acid to a surface of another support. If desired, an intermediate paper prepared by applying a solid acid to a surface of a support and microcapsules containing a color former to the other surface thereof may be employed. The second type of copying paper consists of a support which has been coated with both a solid acid and microcapsules (as mentioned above) to a surface of a support.

In using the first type of paper comprising the combination of an upper paper and a lower paper or the combination of an upper paper, an intermediate paper and a lower paper, they are superimposed in such a manner that the microcapsule layer and solid acid layer come into contact with each other. When a localized pressure is applied to the combination, the microcapsules present in the area under pressure are broken, and the color former liberated from the microcapsules reacts with the solid acid to form a color dye. Similarly, in the case of using a pressure sensitive copying paper of the type having the microcapsules and solid acid on the same surface of the support, the paper forms color dye in the areas to which pressure is applied.

Hitherto, there has not been known any colorless compound which by itself will form a reddish purple color on reaction with an electron acceptor. However, as substantially colorless compounds which will by themselves form magenta color on reaction with an electron acceptor there are known Rhodamine B-Anilinolactam and Rhodamine B-P-Chloroanilinolactam as disclosed in U.S. Pat. NO. 2,695,245. These compounds, however, are slow in color-forming speed and have poor fastness to light after color-forming. As compounds which are initially yellow and instantly develop magenta there are known Rhodamine B-P-nitroanilinolactam as disclosed in U.S. Pat. NO. 2,695,245 and 2-(4-N,N-diethylaminostyryl)-3,3-dimethyl-3H-indole as disclosed in Japanese Pat. No. 21033/1966, but these are poor in fastness to light, both before and after color-forming.

An object of the present invention is to provide a pressure sensitive copying paper which will form a reddish purple color by incorporating into the microcapsule the compound represented by the general formula set out below.

Another object of the present invention is to provide a pressure sensitive copying paper which will form black, blue-black or other desired hues by combination of the compound described below with any of the known yellowish-orange or blue color formers.

We have found that by using a compound represented by the general formula



(wherein  $R_1$  and  $R_2$  each represents an alkyl group having one to five carbon atoms or a benzyl group, and  $X_1$ ,  $X_2$ ,  $X_3$  and  $X_4$  each represents a hydrogen atom, a halogen atom, an alkoxy group, or a methyl group), as a color-former, there is obtained a pressure sensitive copying paper which will form a reddish purple color, or by combination with any of the known yellowish-orange or blue color formers, will form black, blue black or other desired hue. The pressure sensitive copying paper containing a compound of the above general formula in accordance with the present invention has a very high stability in air before color-forming, and consequently, does not discolor and does not lose its color-forming property during storage. It instantly forms the deep reddish purple color and is very excellent in fastness to light, heat resistance and water resistance after color-forming. In addition, it is not desensitized by admixture with the known yellowish-orange or blue color developers.

The compound represented by the above general formula which will form reddish purple color is exemplified by the following compounds:



The compound of the above formula used in the present invention may be prepared by reacting 2-(4'-dialkylamino-2'-hydroxybenzoyl) benzoic acid with a corresponding thioindoxyl at a reaction temperature of 30° to 100° C. for 1 to 24 hours in a 60-98 percent sulfuric acid. After being cooled to room temperature, the reaction mixture is poured into a large quantity of ice water, and the resulting precipitate is recovered by filtration and treated with an aqueous alkali to obtain a compound of the above general formula.



The structure of the compounds obtained by the foregoing reactions has been established by infrared ray absorption spectrum analysis and elementary analysis. With respect to the compounds thus obtained, an absorption band in the neighborhood of 1,750  $cm^{-1}$  is observed which is a characteristic absorption bond for carbonyl in a lactone ring. No other absorption bond for carbonyl and hydroxyl groups is observed. The results of the elementary analysis coincide with the theoretical values as indicated by the following examples in which the manufacture of typical compounds represented by the above general formula is illustrated.

#### SYNTHESIS EXAMPLE 1

Manufacture of the color former (1),  $R_1=R_2=Et$ ,  $X_1=X_2=X_3=H$  and  $X_4=OEt$  in the general formula.

15.7 g. (1/21 mole) of 2-(4'-diethylamino-2'-hydroxybenzoyl) benzoic acid and 9.7 g. (1/21 mole) of 6-ethoxythioindoxyl were dissolved in 30 g. of a 96 percent sulfuric acid at a temperature below 40° C. and reacted at (90±2)° C. for 3 hours. After being cooled to room temperature, the liquid reaction mixture was poured into 500 g. of ice water and the precipitate was separated by filtration. The precipitate was then extracted with 300 cc. of chloroform while neutralizing with an aqueous caustic soda. The resulting chloroform solution was washed several times with water and condensed under reduced pressure, and the thus precipitated crystal was recrystallized from a solution in a mixture of benzene and ligroin to obtain 18.6 g. of a colorless crystal having a melting point of 194-196° C.  $\lambda_{max}=570m\mu$  (95 percent acetic acid).

The crystal had the following composition:

$C_{28}H_{25}O_4NS$  C: 71.31 (71.24), H: 5.34 (5.36), N: 70.297 (2.89).

The numerical values outside the parentheses are the measured values and those within parentheses are the theoretical values in percent. The data of elementary analysis is similarly indicated in the following examples.

#### SYNTHESIS EXAMPLE 2

Manufacture of the color developer (2),  $R_1=R_2=Et$ ,  $X_1=Me$ ,  $X_2=X_3=H$  and  $X_4=Cl$  in the general formula.

15.7 g. (1/21 mole) of 2-(4'-diethylamino-2'-hydroxybenzoyl) benzoic acid and 9.9 g. (1/21 mole) of 6-chloro-4-methoxythioindoxyl were reacted and treated in the same manner as in example 1, and the precipitate was recrystallized with acetone to obtain 17.8 g. of a colorless crystal having a melting point of 234-235° C.,  $\lambda_{max}=573m\mu$  (95 percent acetic acid).

The crystal had the following composition:

$C_{27}H_{22}O_3NSCl$  C: 68.13 (68.21), H: 4.66 (4.63), N: 2.94 (2.91).

15

#### SYNTHESIS EXAMPLE 3

Manufacture of the color developer (3),  $R_1=Me$ ,  $R_2=benzyl$ ,  $X_1=X_3=Cl$  and  $X_2=X_4=H$  in the general formula.

18.1 g. (1/21 mole) of 2-(4'-N-benzyl-N-methylamino-2'-hydroxybenzoyl) benzoic acid and 11.0 g. (1/20 mole) of 4,7-dichlorothioindoxyl were dissolved in 40 g. of a 90 percent sulfuric acid at a temperature below 40° C. and thereafter reacted at (95±2)° C. for 4 hours and treated in the similar manner as in example 1 to obtain 21.4 g. of a colorless crystal having a melting point of 224-226° C.,  $\lambda_{max}=574m\mu$  (95 percent acetic acid).

The crystal had the following composition:

$C_{33}H_{19}O_3NSCl_2$  C: 68.70 (68.58), H: 3.65 (3.53), N: 2.67 (2.58).

30

#### SYNTHESIS EXAMPLE 4

Manufacture of the color developer (4),  $R_1=Et$ ,  $R_2=benzyl$ ,  $X_1=X_3=H$ ,  $X_2=Cl$  and  $X_4=Me$  in the general formula.

18.8 g. (1/21 mole) of 2-(4'-N-benzyl-N-ethylamino-2'-hydroxybenzoyl) benzoic acid and 9.9 g. (1/20 mole) of 5-chloro-7-methyl-thioindoxyl were treated in the similar manner as in example 1 to obtain 19.3 g. of a colorless crystal having a melting point of 203-205° C.,  $\lambda_{max}=573m\mu$  (95 percent acetic acid).

The crystal had the following composition:

$C_{33}H_{21}O_3NSCl$  C: 71.42 (71.51), H: 4.49 (4.42), N: 2.60 (2.56).

40

#### SYNTHESIS EXAMPLE 5

Manufacture of the color developer (5),  $R_1=Et$ ,  $R_2=benzyl$ ,  $X_1=X_2=X_3=X_4=H$  in the general formula.

18.8 g. (1/20 mole) of 2-(4'-N-benzyl-N-ethylamino-2'-hydroxybenzoyl) benzoic acid and 7.4 g. (1/20 mole) of thioindoxyl were dissolved in 41 g. of a 80 percent sulfuric acid at a temperature below 40° C., then reacted at (90±2)° C. for 3 hours and treated in the similar manner as in example 1 to obtain 17.5 g. of a colorless crystal having a melting point of 166-168° C.,  $\lambda_{max}=572m\mu$  (95 percent acetic acid).

The crystal had the following composition:

$C_{33}H_{23}O_3NS$  C: 76.07 (76.14), H: 4.73 (4.80), N: 2.86 (2.81).

50

For the manufacture of pressure sensitive copying papers using as a color former the compound represented by the general formula in accordance with the present invention, there may be adopted such methods well known in the art as disclosed in U.S. Pat. Nos. 2,548,366, 2,800,457, and 2,800,458, i.e., the method of preparing microcapsules making use of the phenomenon of complex coacervation.

The present invention is characterized by the use of the compound represented by the above general formula as a color former, and the characteristics of the pressure sensitive copying paper in accordance with the present invention are not varied significantly by the method employed for the manufacture thereof.

The color former may be used in the amount of 0.5 to 5 percent by weight of the organic solvent.

The electron acceptive solid acid used in the pressure sensi-

75

tive copying paper in accordance with the present invention includes a clay substance such as acid clay, active clay, atapalgite, zeorite or bentonite, and solid organic acid, such as succinic acid, tannic acid, pyrogallol, pentachlorophenol or phenolic resin. The organic solvent for dissolving the color former includes ethylene glycol, chlorinated benzenes and chlorinated diphenols.

Some embodiments of the present invention will now be illustrated by the following examples in which there were used compounds represented by the above general formula as color formers.

#### EXAMPLE 1

3 g. each of the color formers (1 to 5) was separately dissolved in 100 g. of trichlorodiphenyl, and 20 g. of gum arabic, and 160 g. of water added to and the resulting solution emulsified at 50° C.

To the emulsion thus obtained there were added 20 g. of an acid-treated gelatin and 160 g. of water, then added thereto with stirring, acetic acid to adjust the pH of the emulsion to 5. To the emulsion there was then added 500 g. of water to promote coacervation and, after formation of a film of a concentrated liquid gelatin-gum arabic mixture around each particle of the trichlorodiphenyl containing the color former dissolved therein, the pH of the emulsion was adjusted to 4.4, and 3.8 g. of a 37 percent formalin was added to the emulsion to harden said liquid film on the particles of trichlorodiphenyl. Thereafter, the emulsion was cooled to 10° C., added with an aqueous sodium hydroxide to adjust its pH to 9 allowed to stand still for 5-6 hours to complete capsulation. The encapsulated liquid mixture was then applied to a paper by, e.g., roll coating, air knife coating or like coating manner and dried. When the coated paper thus obtained (upper paper) was superimposed on a paper which had been coated with an electron acceptive solid acid such as acid clay, active clay, atapalgite, georite, or bentonite in the manner such that the coated surface of the upper coated came into contact with the coated paper of the clay-coated paper and a hand-writing pressure or impact pressure of a typewriter key was imposed thereto, a deep color was instantly formed on the pressed areas of the lower clay coated paper. The color formed was reddish purple in all cases regardless of the particular color former and clay used. The thus formed color faded little when exposed to direct sunlight for a long period of time, and faded little when wetted with water. Similar reddish purple color forming was also attained in the case where there was used a lower paper coated with an organic solid acid such as succinic acid, pyrogallol, para-toluenesulfonic acid, pentachlorophenol or phenolic resin in place of the clays. No deterioration in color forming property was observed even where the upper papers thus obtained were heated at 100° C. for 20 hours or exposed to sunlight for a long period of time.

#### EXAMPLE 2

An upper paper was prepared in the same manner as in example 1 except that there was used 1.0 g. of the color former

(2) in combination with 0.5 g. of Benzoyl Leuco Methylene Blue, 0.7 g. Malachite Green Lactone, 0.3 g. of Crystal Violet Lactone, and 1.2 g. of 2-(4-acetamidostyryl)-3,3-dimethyl-3H-indole all of which are well-known color formers. There was instantly formed black color on the lower paper when the upper paper thus formed was superimposed on the lower paper having been coated with an electron acceptive solid acid and a handwriting pressure was imposed thereto.

10 A pressure-sensitive copying paper obtained by treating a paper in the same manner as in example 1 except that there was used 0.7 g. of the color former (1) in combination with 0.5 g. of Benzoyl Leuco Methylene Blue, 2.0 g. of Chrystal Violet Lactone, and 0.3 g. 2-(4-acetamidostyryl)-3,3-dimethyl-3H-indole. There was instantly formed a blue black color on the lower paper when the upper paper thus formed was superimposed on the lower paper having been coated with an electron acceptive solid acid and a hand-writing pressure imposed thereto.

#### EXAMPLE 4

The encapsulated liquid mixture as in example 1 was applied to a clay-coated paper. The pressed areas of the dual-coated paper thus obtained formed colors similar to those as in Example 1.

What is claimed is:

1. A pressure sensitive copying paper comprising a support having coated thereon microcapsules containing an organic solvent solution of a substantially colorless compound represented by the following formula:



wherein R<sub>1</sub> and R<sub>2</sub> each represents a member selected from the group consisting of an alkyl group having one to five carbon atoms and a benzyl group, and X<sub>1</sub>, X<sub>2</sub>, X<sub>3</sub>, and X<sub>4</sub> each represents a member selected from the group consisting of a hydrogen atom, a halogen atom, an alkoxy group and a methyl group which in coming into contact with an electron acceptable solid acid forms a color dye.

2. The pressure sensitive copying paper as claimed in claim 1 wherein said electron acceptable solid acid is a member selected from the group consisting of acid clay, active clay, atapalgite, zeolite, bentonite, succinic acid, tannic acid, pyrogallol, pentachlorophenol and phenolic resin.

\* \* \* \* \*